

Feb. 10, 1959

R. P. WEEGAR ET AL

2,873,207

DIAZOTYPE REPRODUCTION MATERIAL AND METHOD

Filed Feb. 21, 1955



INVENTORS:

RALPH P. WEEGAR  
HENRY C. UNKAUF

BY

*Margalef, Johnston, Cook & Root*

ATT'YS

# United States Patent Office

2,873,207

Patented Feb. 10, 1959

1

2,873,207

## DAZOTYPE REPRODUCTION MATERIAL AND METHOD

Ralph P. Weegar, Villa Park, and Henry C. Unkauf, Chicago, Ill., assignors to Eugene Dietzgen Co., Chicago, Ill., a corporation of Delaware

Application February 21, 1955, Serial No. 489,439

12 Claims. (Cl. 117—34)

This invention relates to a diazotype reproduction material and method of manufacture. More particularly, it relates to the provision of a light-sensitive diazotype layer on an impervious organic surface of a photographic base material, especially in the production of a dimensionally stable photographic reproduction material.

Water and organic solvent-impervious organic surfaces such as those on polyester-filled glass and cotton fabrics, as commonly employed in the form of sheets in the drafting and printmaking field, pose difficult problems in the application and fixation thereon of other substances, particularly materials which provide photographic light-sensitive layers.

In the provision of photographic light-sensitive layers on base materials, an absorbent surface is commonly treated with a solution of light-sensitive components which serve to reproduce a desired image. Thus, for example, diazotype reproduction media are produced by treating an absorbent surface with a solution containing azo dye components in an uncombined form. The most commonly used base material is paper, and the components are usually in aqueous solution. Sufficient penetration is obtained to insure bonding of the paper and the sensitizing composition, and the ultimate dye image. Cellulose esters and ethers are also in common use as base materials, and they are impregnated with a sensitizing solution by the addition of penetrating or swelling agents which have a solvent action on the base material, to insure the necessary bonding.

The prior methods are, however, unsuitable for coating or impregnating water and organic solvent-impervious surfaces, there being insufficient bonding with the base material to provide a uniform layer of the sensitizing components which is permanently bonded and is resistant to wear and abrasion. Furthermore, the dye images reproduced on the surface by exposure and development have little permanency, and in order to prevent easy removal of the images, it is necessary to overcoat them with a transparent coating. Even such a coating on, for example, polyester-impregnated glass cloth, is easily scratched, chipped and otherwise damaged in ordinary handling, shipping, and storage.

There are a number of advantages in the use of water and organic solvent-impervious base materials, especially those having a polyester surface, and it is therefore highly desirable to provide reproduction materials which include these materials together with a light-sensitive layer.

It is therefore an object of the invention to provide a new and improved diazotype reproduction material and method of manufacture.

A particular object is to provide a reproduction material which includes a base having a polyester surface and a light-sensitive diazotype layer thereon.

A further object is to provide a dimensionally stable diazotype reproduction element which furnishes excellent uniform permanent reproduction and which is resistant to the various conditions encountered.

An additional object is to supply a reliable and effective

2

method for providing a light-sensitive diazotype layer on a liquid-impervious polyester surface of a photographic base material. The impervious surface referred to absorbs substantially no water or organic solvent, so that it is un receptive to aqueous and organic solvent solutions, for all practical purposes, and there will be no or only insubstantial adherence or binding of the solutions and their ingredients to the surface.

Another object is to coat an impervious polyester surface employing a principally non-aqueous organic solvent solution of a light-sensitive diazo compound.

Still another object is to provide a diazotype reproduction material having a base of a polyester-filled tracing cloth, such as a polyester-filled glass or cotton fabric, and the like, and a strongly adherent diazotype layer. Polyester-filled glass tracing cloth, commonly referred to as photo-template glass cloth, provides a dimensionally stable reproduction material.

An additional object is to provide a method of preparing a polyester surfaced body having a design on the surface.

Yet another object is to provide a diazotype coat on a photographic base material having the desired properties of transparency or translucency, little color, storage stability and resistance to chemical and physical attack under the conditions normally encountered.

Other objects include the manufacture and application of new and improved coating compositions, and coats and coated base materials, and the provision of new and useful methods. These and other objects and advantages of the invention will appear on consideration of the specification taken in conjunction with the attached drawing, in which the single figure is a broken perspective view of photo-template glass cloth provided with a diazotype layer or coat, according to a preferred embodiment of the invention.

The invention provides a photographic reproduction material which includes a base material having an impervious unsaturated polyester resin surface, and a coat of a light-sensitive diazo compound and a cellulose ester or ether. To furnish a satisfactory bond with the polyester surface, a bonding coat of an amine-formaldehyde resin is included between the polyester surface and the diazo layer or coat.

A method for providing a diazotype layer on an impervious unsaturated polyester resin surface is provided in the invention, which method includes providing on the polyester surface a coat of an amine-formaldehyde resin and a solvent-soluble material serving to increase the solvent sensitivity of the coat while retaining its adhesiveness, and coating the resulting coated surface with an organic solvent solution of a diazo compound and a cellulose ester or ether.

The base material provided with a coat of an amine-formaldehyde resin forms the subject matter of copending application, Serial No. 489,438, filed February 21, 1955, by Ralph P. Weegar and Henry C. Unkauf, which is incorporated herein by reference and made a part hereof as fully as if set forth herein in its entirety.

As disclosed in the above copending application, it has been found that amine-formaldehyde thermosetting resins exhibit very good adhesion to polyesters, in particular, polyester-filled fabrics, such as glass or cotton fabrics, represented by the tracing cloths in common use in the drafting and printmaking field.

The invention has particular reference to the unsaturated polyester resins, as the class is defined on pages 520-524 of Modern Plastics Encyclopedia, issue/vol. 32, No. 1A, 1954. These resins are condensation products of dibasic acids and glycols, prepared in part from an unsaturated dibasic acid, such as maleic or fumaric acid, and a glycol, such as ethylene glycol. The linear polyester is

cross-linked with a polymerizable monomer, a monomeric vinyl type compound such as vinyl acetate, methyl methacrylate and styrene, to provide a thermoset solid. Illustrative of the polyester resins coated in the invention are the Paraplex polyester-styrene resins (Resinous Products & Chemical Co.), such as P-13 (flexible grade), P-43 (rigid grade) and P-47 (semi-rigid grade). In the preparation of flexible tracing cloth, an exemplary composition for filling the fabric is a mixture of P-13 and P-47 in a weight ratio on the order of 1 to 4. These impervious polyester materials are resistant to the conditions encountered in the production and use of photographic reproduction media.

The amine-formaldehyde resin may be a melamine, urea, urea-melamine, alkylated urea, acetylene diurea, or triazine type formaldehyde resin, for example. Preferably, a urea-modified melamine formaldehyde type resin is employed, such as Uformite MU-56 (Resinous Products & Chemical Co.). Other representative resins are Uformite MM-55, a melamine resin, and MX-61, a triazine type resin. The resins are employed in heat-convertible form and are cured or thermoset on the polyester surface.

The cured amine-formaldehyde resin may be and frequently is resistant to the solvents which it is desired to use in the subsequent application of a photographic sensitizing composition, such as alcohols, ketones and esters, and incompatible with the other constituents of the sensitizing composition. The resin is therefore modified to provide a coating to which a sensitizing layer will adhere properly without destroying the adhesion to the polyester surface. Thus, in addition to the amine-formaldehyde resin, the coating composition and resulting coat according to the invention include a solvent-soluble material serving to increase the solvent sensitivity of the coat while retaining its adhesiveness. The preferred solvent-soluble materials are the esters and ethers of cellulose, such as cellulose nitrate, ethyl cellulose, and cellulose acetate, and shellac.

The resin coating compositions contain the described ingredients in solution in a suitable volatile organic solvent, lower aliphatic esters being preferred as exhibiting good compatibility. The compositions should also include a curing catalyst, such as an acid. The base material is coated and thus rendered receptive to the sensitizing composition by applying the solution to the surface of the material, removing solvent, and curing, preferably at a temperature of about 220-300° F.

It is further preferred to overcoat the amine resin coat, to increase its receptivity to the outer diazo-containing coat. The overcoat contains shellac and a member of the class of cellulose ethers and esters, such as ethyl cellulose, cellulose acetate, and nitrocellulose. The overcoat is applied in volatile organic solvent solution, e. g., in a lower aliphatic alcohol or ester, the solvent is removed, and the overcoat is cured, preferably at 220-300° F. Both the first coat and the overcoat are preferably cured together.

The sensitizing composition may be applied at any time after the overcoat, as described in more detail subsequently. The sensitized product prepared in this manner will then consist essentially of the base material and three coats, films or layers on a surface thereof. It will be understood that these coats will merge and extend into adjacent areas at their inner faces due to penetration, diffusion, and the like during application and curing or hardening.

While the proportions of the components of the amine resin or first coatings are subject to some variation depending upon the particular components and the properties sought, it is preferred that the amine-formaldehyde resin be present in a major proportion of the content of the amine resin and solvent-soluble material. Preferably, the solvent-soluble material, e. g., cellulose ester, cellulose ether or shellac, is present in a proportion of about

15-80% by weight of the amine resin, and it is further preferred that the proportion be about 15-60%.

To improve the properties of the amine-formaldehyde resin coating, an alkyd resin, in particular, a non-oxidizing pure phthalic alkyd resin, may be incorporated into the compositions. The alkyd resins are preferably cured or thermoset pure phthalic alkyd resins modified with a non-drying oil acid, especially those of the glycerol-phthalic anhydride type. Thus, for example, the alkyd resins may be the reaction products of phthalic acid or halogenated phthalic acid with a trihydric alcohol such as glycerol or other alcohols having three or more hydroxyl groups, or their hydroxyalkyl ethers, modified with a non-drying oil acid such as the acids of coconut oil, castor oil, cottonseed oil, olive oil, and the like. The preferred resin is a cured coconut oil acid-modified glycerol phthalate resin. When the alkyd resin is mixed with the heat-convertible amine-formaldehyde resin and the mixture is cured on the polyester surface, the resins adhere strongly and have a very pale color which is retained during and after curing.

In this preferred composition, the alkyd resin is employed in an amount equivalent to about 50-200% by weight of the amine-formaldehyde resin, depending on the particular properties sought. An especially advantageous coat on phototemplate glass cloth is obtained when about 150-200% by weight of alkyd resin is used, based on the amine resin. Employing both resins, the proportion of solvent soluble material is as described above for the amine resin alone, but the proportion is based instead on the combined weight of the alkyd and amine resins.

In the above first overcoat, which is applied over the amine resin or amine resin-alkyd resin coat, shellac is the predominant ingredient, about 10-50% by weight based on the shellac of cellulose ester or ether being included, with 15-25% of the latter being further preferred.

It may also be of advantage to provide a second overcoat, on the surface of the first and between it and the sensitizing coat. This embodiment is that illustrated in the drawing. The second overcoat contains an acrylic ester resin and a cellulose ester or ether, preferably nitrocellulose. The most useful acrylic esters are the methyl and ethyl esters of acrylic acid and methacrylic acid. The resins employed belong to the class of soft resins soluble in petroleum hydrocarbons. Ethyl acrylate appears to provide the most suitable resin. An exemplary resin is Acryloid F-10 (Resinous Products & Chemical Co.), a mineral thinner soluble acrylic ester resin.

The second overcoat preferably contains a major weight proportion of the cellulose derivative, based on the total of the latter and the acrylic ester resin. It is further preferred that the proportion of acrylic ester resin be about 25-50% by weight based on the cellulose derivative. The second overcoat is applied to the first overcoat, after curing the latter, in a volatile organic solvent solution of the polymerized acrylic ester and the cellulose derivative, preferably in a lower aliphatic ester. The coated material is then dried to remove volatiles, preferably at about 150-175° F.

The polyester surface thus coated and rendered receptive to the sensitizing composition is provided with an outer layer or coating of a light-sensitive diazo compound and a cellulose ester or ether, by applying the components in an organic solvent solution. A clear, colorless film-forming cellulose ether or ester is employed, such as ethyl cellulose, cellulose acetate, and nitrocellulose.

An important phenomenon cooperating in the invention is that although the films of the cellulose derivatives are not alone impervious to ammonia and water vapor, and to the developing solutions, so that a diazo layer cannot be overcoated satisfactorily with them, the thin films are sufficiently pervious when mixed with the diazo com-

ponents to exhibit good developing properties. On the other hand, the films or coats may be regarded as water resistant and have excellent stability to heat, ammonia, water and water vapor, not swelling, loosening or dissolving, and they are very rugged and durable.

Diazo compounds which are organic solvent soluble and suitable for the sensitizing compositions of the invention include, for example, those which are derived from aromatic p-diamines of the benzene series, particularly those which are N-mono or di-substituted on the undiazoized amino groups, with or without aliphatic substitution on the benzene ring. Also included are resinous condensation products of aldehydes, such as formaldehyde, with these light-sensitive diazo compounds, and the p-amino phenyl sulfones of the diazo compounds. The boron trifluoride, the stannous chloride, the cadmium chloride, and the zinc chloride double salts of the aforementioned light sensitive organic solvent soluble diazo compounds are included. Specific examples of such compounds which are used in the production of diazo-type images of high contrast are the diazo derivatives of p-amino-N-methyl aniline, p-amino-N-di-methyl aniline, p-amino-N-ethyl aniline, p-amino-N-di-ethyl aniline, p-amino-N-methyl-N-ethyl aniline, p-amino-N-ethoxy aniline, p-amino-N-methyl-N-ethoxy aniline, p-amino-N-ethyl-N-ethoxy aniline, p-amino-N-diethyl-m-toluidine, and 1-amino-3-methyl-4-ethylamino benzene, all in the form of their diazo double salts with zinc chloride, cadmium chloride, stannous chloride, or boron trifluoride, or their diazo p-amino-phenyl sulfones, or their diazo-formaldehyde resinous condensation products.

As coupling components, any compound which will function as a coupling component may be employed either in the coating composition together with the diazo compound in order to produce a two-component system, or in the developing solution as a color forming developer. In either case, the coupling component selected will be one which will produce the desired color or a combination of coupling components which will produce a multi-color effect. Examples of preferred coupling components are: 2,3-dihydroxy naphthalene and its 6-sulfonic acid derivative, phloroglucinol, methyl phloroglucinol, resorcinol, resorcinol-mono-methyl ether, dichloro resorcinol, m-hydroxy phenyl urea, acetoacetanilide, acetoacetyl-cyclohexyl amide, 7-hydroxy naphthalene-1-biguaniide, 7-hydroxy-1,2-naphthimidazole, 2-amino-8-naphthol-3,6-disulfonic acid, 2,7-dihydroxy naphthalene, 1-naphthol-4-sulfonic acid, and 1-amino-8-naphthol-3,6-disulfonic acid.

The sensitizing compositions may contain the usual adjuncts such as metal salts, to intensify the dyestuff image, i. e., aluminum sulfate, titanium ammonium fluoride, nickel sulfate and the like, and acids designed to retard precoupling such as citric acid, maleic acid, tataric acid, boric acid and the like.

The diazo composition can also advantageously include a filler such as colloidal silica, hydrated silica, diatomaceous earth, bentonite, mica and the like. The filler acts to raise the softening point of the coating, promote development of a print by inducing porosity, and provide a mat surface.

The sensitizing composition is a principally non-aqueous organic solvent solution of the diazo ingredients and the cellulose ester or ether. The ingredients are balanced for mutual compatibility and the properties desired. The solvent and cellulose derivative are selected for solubility and are adjusted to a viscosity suitable for application and which will properly suspend the filler, and to provide a continuous flexible abrasion-resistant film. The solvents are preferably selected from the group of lower aliphatic alcohols, lower aliphatic ketones, lower aliphatic glycol esters and lower aliphatic glycol ethers, and they are specially selected to furnish a controlled rate of drying on application to the base material. Thus, the solvents are balanced to result in a drying rate

which is slow enough to avoid condensation or pickup of water and to avoid premature drying in the rollers or other equipment, yet rapid enough to dry rapidly and completely in a satisfactory manner after application, furnishing a thin uniform strongly adhering and non-tacky surface coat. For example, a drying rate of 5-10 minutes at 150-175° F. in commercial coating equipment is provided.

The primary solvent for the mixture is methanol or ethanol, or acetone or methyl ethyl ketone may be substituted in whole or in part. The primary solvent is present in a major proportion by weight of the total of the organic solvents, preferably in a proportion of 60-90% of the solvents. The primary solvent is blended with a minor proportion, preferably 10-40%, of a higher boiling alcohol or the equivalent, which serves to prevent overly rapid drying with consequent "blushing." The medium boiling lower aliphatic alcohols having 4 carbon atoms or more and which are liquid at room temperature, such as butyl alcohol and amyl alcohol, are desirably employed, and they may be substituted in whole or in part by lower aliphatic glycol esters or ethers, such as the esters or ethers of ethylene glycol, propylene glycol and glycerine. In a controlled low humidity, normal or isopropanol may be used alone. In the selection of solvents, due consideration must be given to the solubility of the cellulose derivative.

A preferred combination of solvents for application with ethyl cellulose and nitrocellulose is a mixture of 90-85% of methanol and 10-15% of butanol, or an equivalent mixture. With cellulose acetate, a ketone or an ester should be included.

In the compositions which are ammonia developed after printing, a small amount of a lower aliphatic glycol, such as ethylene glycol, propylene glycol and glycerine, may be included to assist in picking up water vapor in developing. The proportion of glycol is preferably about  $\frac{1}{4}$  to 1 part by weight to 1 part of the cellulose derivative. This function together with that of the secondary or higher boiling solvent is also provided by cellosolve esters, such as the lower aliphatic cellosolve esters, preferably  $\beta$ -alkoxy ethyl acetate.

In the sensitizing composition, the cellulose ether or ester binder is preferably employed in a proportion of about  $\frac{1}{4}$  to 5 parts by weight to 1 part of diazo compound. The reference to diazo compound does not include the coupling components and the adjuncts. About 20 to 200 parts by weight of solvent are employed per part of diazo compound, so that the diazo compound is present in a proportion of about 5 to 0.5% of the solvents.

About 30 to 60 parts of solvent per part of the cellulose binder are employed, equivalent to a proportion of binder of about 3.3% to 1.6% based on the solvents. It is ordinarily preferred to incorporate about 0.5 to 5 parts of filler per part of diazo compound.

The composition includes merely sufficient water to dissolve those components of the diazo system which are insoluble or difficultly soluble in organic solvents, but not enough to precipitate the cellulose ester or ether binder, and the proportion of water thus amounts to a maximum of about 3% by weight of the complete sensitizing composition.

The sensitizing composition prepared in the above manner is applied to the polyester surface which has been rendered receptive thereto by the application of the described amine-formaldehyde resin coat, by brushing, spraying, bead-coating, roller coating, silk screening, or the like, to provide a thin coat on the surface. The material is dried in the dark, at a temperature of from about room temperature to about 250° F., the upper temperature being limited by the stability of the diazo components. An adherent sensitized layer is thus firmly bonded to the polyester surface. The photographic reproduction material so produced can be exposed to light of varying intensity in accordance with a design to be reproduced

thereon, e. g., under a pattern to be reproduced, and the images developed by exposure to ammonia vapors in the case of the two-component or dry-developing process, or by spraying, dipping, swabbing or sponging with a developing solution in the case of the one-component or moist-developing process.

When the original pattern or drawing is produced on a dimensionally stable medium, such as photo-template glass cloth, the final diazotype reproduction will be an exact true-to-scale duplicate copy of the original. The resulting copy is unaffected by atmospheric moisture and continues to maintain its dimensional stability during handling and storage. The duplicate copy requires no over-spraying or lacquering, as there is no rubbing or peeling off of the surface, and the image is well protected. The reproduction materials and the resulting prints may be transported and employed in various localities, for example, they have found widespread application in the manufacture of metal templates in the aircraft industry.

The following examples are furnished to assist in providing a complete understanding of the invention, but it is to be understood that the invention is not limited thereto nor to the specific compositions, proportions and conditions set forth therein, which are given only for purposes of illustration.

#### Example 1

The following composition is employed to provide an amine-formaldehyde resin layer on an impervious polyester surface:

|                                                       |    |        |
|-------------------------------------------------------|----|--------|
| Urea - melamine - formaldehyde resin (Uformite MU-56) | gm | 130    |
| 5-6 Second RS nitrocotton                             | gm | 20-100 |
| Ethyl acetate                                         | cc | 900    |
| n-Butyl acetate                                       | cc | 100    |
| Phosphoric acid                                       | gm | 4      |

The composition is brushed, sprayed, roller coated or applied in other similar fashion to a surface of an unsaturated polyester resin photographic base material, the coated material is dried to remove the volatiles, for example, at about 150-175° F. for about 5 minutes, and the coat is cured by heating for about 5 minutes at 250-300° F.

#### Example 2

Another exemplary composition is the following:

|                                                   |    |        |
|---------------------------------------------------|----|--------|
| Urea-melamine-formaldehyde resin (Uformite MU-56) | gm | 130    |
| Ethyl cellulose                                   | gm | 20-100 |
| Ethyl acetate                                     | cc | 900    |
| n-Butyl acetate                                   | cc | 100    |
| Phosphoric acid                                   | gm | 4      |

The coat is applied as in Example 1 and is cured for about 5 minutes at 250-300° F.

#### Example 3

An additional composition wherein an alkyd resin is included, is the following:

|                                                               |    |        |
|---------------------------------------------------------------|----|--------|
| Cured, non-drying oil acid-modified pure phthalic alkyd resin | gm | 130    |
| Urea-melamine-formaldehyde resin                              | gm | 50-130 |
| 1/2 second RS nitrocotton                                     | gm | 50-150 |
| Ethyl acetate                                                 | cc | 900    |
| n-Butyl acetate                                               | cc | 100    |
| Ethyl phosphoric acid                                         | gm | 8      |

The coat is applied as in Example 1 and is cured for about 5 minutes at 250-300° F.

#### Example 4

The following is an example of a composition for providing an overcoat on the surface of the coat formed according to Examples 1-3:

|                           |    |       |
|---------------------------|----|-------|
| Bleached, dewaxed shellac | gm | 125   |
| 5-6 Second RS nitrocotton | gm | 15-50 |
| Ethyl acetate             | cc | 200   |
| Methanol                  | cc | 700   |
| n-Butanol                 | cc | 100   |

The composition is preferably applied to the surface of the first coat after drying and before curing the coat. The overcoat is then dried in the same manner, and the combined coatings are cured together at about 250-300° F. for about 5 minutes.

#### Example 5

Another example of a composition for providing an overcoat to further increase the receptivity of the alkyd resin coat is as follows:

|                           |    |       |
|---------------------------|----|-------|
| Bleached, dewaxed shellac | gm | 125   |
| Ethyl cellulose           | gm | 15-50 |
| Ethyl acetate             | cc | 200   |
| Methanol                  | cc | 700   |
| n-Butanol                 | cc | 100   |

#### Example 6

The following composition is applied by roller coating 25 commercial photo-template glass cloth with a layer which is 0.0002-0.0004" thick.

|                                                                                                                                 |    |     |
|---------------------------------------------------------------------------------------------------------------------------------|----|-----|
| Cured coconut oil-modified trihydric alcohol-phthalic anhydride alkyd resin (Duraplex ND-77B, Resinous Products & Chemical Co.) | gm | 130 |
| Urea-melamine-formaldehyde resin (Uformite MU-56)                                                                               | gm | 75  |
| 5-6 Second RS nitrocotton                                                                                                       | gm | 75  |
| Hydrated silica                                                                                                                 | gm | 50  |
| Ethyl acetate                                                                                                                   | cc | 900 |
| n-Butyl acetate                                                                                                                 | cc | 100 |
| Ethyl phosphoric acid                                                                                                           | gm | 10  |

The cloth so coated is dried at about 150-175° F. for five minutes to remove the volatiles, resulting in a sheet of photo-template cloth 1 as illustrated in the drawing, having an amine resin-alkyd resin coat 2 on one surface thereof. At this stage, the coat 2 is uncured, and its adhesion and hardness are not fully developed.

A shellac overcoat 3 is next applied to the outer surface of the resin coat 2 in the same manner in a layer of the same thickness, employing the following composition:

|                           |    |     |
|---------------------------|----|-----|
| Bleached, dewaxed shellac | gm | 100 |
| 5-6 Second RS nitrocotton | gm | 20  |
| Hydrated silica           | gm | 50  |
| Ethyl acetate             | cc | 200 |
| Methanol                  | cc | 700 |
| n-Butanol                 | cc | 100 |

The overcoated product is dried at about 150-175° F. for five minutes, and the combined coatings are cured at about 250-300° F. for five minutes.

The resulting coated photo-template glass cloth is receptive to a light-sensitive diazotype organic solvent composition, which is applied thereover as described in the subsequent examples.

#### Example 7

A second overcoat may be applied on the surface of the first overcoat of Example 6. The following composition is applied and dried in the same manner as the first overcoat:

|                                                                      |    |         |
|----------------------------------------------------------------------|----|---------|
| Mineral thinner soluble acrylic ester resin (Acryloid F-10)          | gm | 5-20    |
| 5-6 Second RS Nitrocotton                                            | gm | 20-40   |
| Ethyl acetate                                                        | cc | 600-800 |
| n-Butyl acetate                                                      | cc | 100-300 |
| β-methoxy ethyl acetate (Carbide & Carbon methyl cellosolve acetate) | cc | 100-300 |

The resulting coated photo-template glass cloth is receptive to a light-sensitive diazotype organic solvent composition, which is applied thereover as described in the subsequent examples. The complete photographic reproduction material or element, illustrated in the drawing, then includes the sheet of photo-template cloth 1, the amine resin-alkyd resin coat 2 adhering to a surface of the cloth, the intermediate shellac first overcoat 3 adhering to the outer surface of the resin coat 2, the intermediate acrylic ester resin second overcoat 4 adhering to the outer surface of the shellac overcoat 3, and the outer sensitizing coat 5 adhering to the outer surface of the acrylic ester resin coat 4. The acrylic ester resin second overcoat 4 may be omitted, so that the sensitizing coat 5 adheres to the outer surface of the shellac overcoat 3.

#### Example 8

This example illustrates the production of a direct (positive image) dimensionally stable sepia intermediate (second original) print, ammonia developed, on photo-template glass cloth.

A solution of sensitizer is prepared, having the following composition:

|                                                                     |     |      |
|---------------------------------------------------------------------|-----|------|
| Methanol                                                            | cc  | 7000 |
| n-Butanol                                                           | cc  | 500  |
| Water                                                               | cc  | 300  |
| Propylene glycol                                                    | cc  | 300  |
| Tartaric acid                                                       | gms | 150  |
| Zinc chloride                                                       | gms | 150  |
| Thiourea                                                            | gms | 150  |
| Resorcinol                                                          | gms | 150  |
| p-Diazo-N-methyl-N-hydroxy-ethyl aniline, zinc chloride double salt | gms | 200  |

These ingredients, thoroughly mixed and filtered, are added to the following mixture:

|                                                 |     |      |
|-------------------------------------------------|-----|------|
| Methanol                                        | cc  | 8000 |
| n-Butanol                                       | cc  | 1600 |
| Silica aerogel (Monsanto Santocel CX)           | gms | 600  |
| 10% ethyl cellulose in methanol (Hercules N-50) | cc  | 6000 |

The final sensitizing solution is stored in a covered crock until ready for use.

A roll of commercial plastic-impregnated photo-template glass cloth, 36" wide, 0.005" thick, 200 yards long, is sub-coated according to Example 6 or 7 and is then bead-coated in a layer about 0.0001-0.0002" thick with the above-described sensitizing solution on a cloth lacquering machine of conventional design, dried in the dark, and wrapped and packaged in 20 yard length rolls. Using part of one of these rolls, a contact print is made by means of a carbon arc light and a vacuum frame, on a 3' x 12' section of the sensitized material. As the original pattern, a 3' x 12' non-dimensioned engineering pencil drawing on plastic-impregnated glass tracing cloth is used.

The resulting sepia intermediate (or second original) print, ammonia developed is an exact, true-to-scale positive copy of the original pencil drawing on glass cloth, having a very small linear distortion. From this "second original" copy can now be made exact true-to-scale non-dimensioned metal template, if the metal has been sensitized with a positive image printing type of sensitizer.

#### Example 9

This example illustrates the production of a direct (positive image) dimensionally stable blue line print, ammonia developed, on photo-template glass cloth.

A solution is prepared, having the following composition:

|           |    |      |
|-----------|----|------|
| Methanol  | cc | 3500 |
| n-Butanol | cc | 250  |
| Water     | cc | 150  |

|                                                                 |     |     |
|-----------------------------------------------------------------|-----|-----|
| Ethylene glycol                                                 | cc  | 150 |
| Citric acid                                                     | gms | 100 |
| Zinc chloride                                                   | gms | 100 |
| Urea                                                            | gms | 100 |
| 5 2,3-di-hydroxynaphthalene                                     | gms | 25  |
| p-Diazo-N-ethyl-N-ethoxy aniline, stannous chloride double salt | gms | 150 |

These ingredients, thoroughly mixed and filtered, are added to the following mixture:

|                                          |     |      |
|------------------------------------------|-----|------|
| Methanol                                 | cc  | 4000 |
| n-Butanol                                | cc  | 800  |
| Hydrated silica                          | gms | 300  |
| Ethyl cellulose 10% solution in methanol | cc  | 3000 |

A roll of plastic-impregnated photo-template glass cloth, 48" wide, 0.005" thick, 150 yards long, is sub-coated according to Example 6 or 7 and is then roller-coated in a layer about 0.0001-0.0002" thick with the above-described sensitizing solution on a cloth lacquering machine of conventional design, dried in the dark, and wrapped and packaged in sheets 4' wide and in lengths from 4' to 12'. A 4' x 8' sensitized sheet is selected, and a print is made from a 4' x 8' "second original" sepia intermediate print on plastic-impregnated glass cloth (made from a non-dimensioned, true-to-scale engineering drawing on photo-template glass cloth by the method described in Example 8).

The resulting blue-line positive copy, printed and ammonia developed, is an exact, true-to-scale positive copy of the "second original" sepia intermediate print, having a very small linear distortion.

#### Example 10

This example illustrates the production of a direct (positive image) dimensionally stable sepia line print, moist developed, on photo-template glass cloth.

A solution is prepared, having the following composition:

|                                                                                |     |      |
|--------------------------------------------------------------------------------|-----|------|
| 40 $\beta$ -Methoxy ethyl acetate (Carbide & Carbon methyl cellosolve acetate) | cc  | 2500 |
| Acetone                                                                        | cc  | 500  |
| n-Butanol                                                                      | cc  | 250  |
| 45 Methanol                                                                    | cc  | 500  |
| Water                                                                          | cc  | 300  |
| Oxalic acid                                                                    | gms | 100  |
| 50 Naphthalene-1,3,6-tri-sulfonic acid, (sodium salt)                          | gms | 200  |
| p-Diazo-N-ethyl-N-benzyl aniline, cadmium chloride double salt                 | gms | 300  |

These ingredients, thoroughly mixed and filtered, are added to the following mixture:

|                                                                    |     |      |
|--------------------------------------------------------------------|-----|------|
| 55 Methanol                                                        | cc  | 2000 |
| Acetone                                                            | cc  | 2000 |
| Silica aerogel (Godfrey L. Cabot "Cab-O-Sil")                      | gms | 300  |
| 60 Cellulose acetate (Hercules, FM grade, 56% acetic acid content) | gms | 150  |

A roll of plastic-impregnated photo-template glass cloth, 42" wide, 0.005" thick, 100 yards long, is sub-coated according to Example 6 or 7 and is then roller-coated with the above-described sensitizing solution on a cloth lacquering machine of conventional design, dried in the dark, and wrapped and packaged in 10 yard length rolls. Using part of one of these sensitized rolls, a contact print is made by means of a carbon arc light and a vacuum frame on a 3 1/2' x 7' section of the sensitized material. A 3 1/2' x 7' non-dimensioned engineering ink drawing on photo-template glass cloth is the "original" employed. The resulting intermediate print is developed by immersion for 1/2 minute in a tank containing

## 11

a developing solution composed of the following ingredients:

|                      |     |      |
|----------------------|-----|------|
| Water                | cc  | 4000 |
| Potassium metaborate | gms | 300  |
| Urea                 | gms | 60   |
| Phloroglucinol       | gms | 10   |
| Resorcinol           | gms | 30   |

After the print is developed, it is rinsed in water and air dried. The resulting sepia line positive print on glass cloth is an exact, true-to-scale positive copy of the original ink drawing on glass cloth, having a very small linear distortion. From this "second original" print can now be made exact, true-to-scale copies on diazo sensitized glass cloth (as described in Example 9), or on metal templates when sensitized with a positive image printing type of sensitizer.

## Example II

This example illustrates the production of a direct (positive image) dimensionally stable black line print, semi-moist developed, on photo-template glass cloth.

A solution is prepared, having the following composition:

|                                                                     |     |      |
|---------------------------------------------------------------------|-----|------|
| $\beta$ -Ethoxy ethyl acetate (Carbide & Carbon cellosolve acetate) | cc  | 2500 |
| Methyl ethyl ketone                                                 | cc  | 500  |
| n-Butanol                                                           | cc  | 250  |
| Methanol                                                            | cc  | 500  |
| Water                                                               | cc  | 300  |
| Diglycolic acid                                                     | gms | 150  |
| Ammonium sulfate                                                    | gms | 150  |
| 4-Diazo-N-benzoyl-2,5-dibutoxy aniline, zinc chloride double salt   | gms | 300  |

These ingredients, thoroughly mixed and filtered, are added to the following mixture:

|                                          |     |      |
|------------------------------------------|-----|------|
| Methanol                                 | cc  | 4000 |
| n-Butanol                                | cc  | 800  |
| Silica Gel, micron sized (Davison)       | gms | 300  |
| 10% ethyl cellulose solution in methanol | cc  | 3000 |

A roll of plastic-impregnated photo-template glass cloth 30" wide, 0.005" thick, and 125 yards long, is sub-coated as described in Example 6 or 7 and is then offset roller-coated with the above-described sensitizing solution on a cloth lacquering machine of conventional design, dried in the dark, and wrapped and packaged in sheets measuring 2 1/2' x 5'. A print is made on one of these sensitized sheets from a 2 1/2' x 5 1/2' "second original" moist-developed sepia intermediate print on photo-template glass cloth produced by the method described in Example 10. For exposure, a carbon arc light is used, and the direct process positive print is made by the contact method, using a vacuum frame. The resulting print is developed by swabbing with a sponge moistened with a developing solution prepared as follows:

|                              |     |      |
|------------------------------|-----|------|
| Water                        | cc  | 1000 |
| Sodium potassium tartrate    | gms | 40   |
| Sodium carbonate (anhydrous) | gms | 30   |
| Sodium thiosulfate           | gms | 40   |
| Phloroglucinol               | gms | 8    |

After the print is developed, it is blotted dry between filter papers, and air dried. The resulting black line semi-moist developed positive print on photo-template glass cloth is an exact, true-to-scale copy of the sepia intermediate print on glass cloth, it having a very small linear distortion.

In the foregoing examples, various combinations of light-sensitive diazo compounds, or light-sensitive diazo compounds and azo coupling components, soluble in the types of organic solvents described, and suitable for the preparation of photographic light-sensitive layers, i. e., which will provide a photographic reproduction, visually

## 12

reproducing a drawing on exposure to light and developing by undergoing a substantial color change, can be substituted for the compounds employed. Likewise, the compositions and procedures can be varied in other ways while still providing the results of the invention and falling within its scope.

In this manner, the invention provides a new and improved diazotype photographic reproduction material, especially a material useful in applications where dimensional stability is required. The new materials are exceptionally versatile in their application, overcome the prior disadvantages and provide new and improved industrial applications.

What is claimed is:

1. The method for providing a light-sensitive diazotype layer on an impervious unsaturated polyester resin surface of a photographic base material which comprises providing on said surface a coat of an amine-formaldehyde resin and a solvent-soluble material serving to increase the solvent sensitivity of the coat while retaining its adhesiveness, providing on said coat an overcoat of shellac and a member selected from the class consisting of cellulose esters and cellulose ethers, and applying to the coated surface a coat of a light-sensitive diazo compound and a member of the class consisting of cellulose esters and ethers.

2. The method for providing a light-sensitive diazotype layer on an impervious unsaturated polyester resin surface of a photographic base material which comprises coating said surface with an organic solvent solution of a heat-convertible amine-formaldehyde resin and a solvent-soluble material serving to increase the solvent sensitivity of the coat while retaining its adhesiveness, removing volatiles, coating the coated surface with an organic solvent solution of shellac and a member selected from the class consisting of cellulose esters and cellulose ethers, curing the coating, and coating the coated surface with an organic solvent solution of a light-sensitive diazo compound and a member of the class consisting of cellulose esters and ethers.

3. The method for providing a light-sensitive diazotype layer on an impervious unsaturated polyester resin surface of a photographic base material which comprises coating said surface with an organic solvent solution of a heat-convertible amine-formaldehyde resin and a cured non-drying oil acid-modified phthalic alkyd resin and a solvent-soluble material from the class consisting of cellulose esters, cellulose ethers and shellac, removing volatiles, coating the coated surface with an organic solvent solution of shellac and a member selected from the class consisting of cellulose esters and cellulose ethers, curing the coatings, and coating the thus coated surface with an organic solvent solution of a light-sensitive diazo compound and a member of the class consisting of cellulose esters and ethers.

4. The method for providing a light-sensitive diazotype layer on an impervious unsaturated polyester resin surface of a photographic base material which comprises providing on said surface a coat of an amine-formaldehyde resin and a non-drying oil acid-modified phthalic alkyd resin and a solvent-soluble material from the class consisting of cellulose esters, cellulose ethers and shellac, a first overcoat of shellac and a number selected from the class consisting of cellulose esters and cellulose ethers, a second overcoat of an acrylic ester resin and a member selected from the class consisting of cellulose esters and cellulose ethers, and an outer coat of a light-sensitive diazo compound and a member of the class consisting of cellulose esters and ethers.

5. The method for providing a light-sensitive diazotype layer on an impervious unsaturated polyester resin surface of a photographic base material which comprises providing on said surface a coat of an amine-formaldehyde resin and a non-drying oil acid-modified phthalic alkyd resin and a solvent-soluble material serving to increase

the solvent sensitivity of the coat while retaining its adhesiveness, providing on said coat an overcoat of shellac and a member selected from the class consisting of cellulose esters and cellulose ethers, and coating the coated surface with an organic solvent solution of a light-sensitive diazo compound and a member of the class consisting of cellulose esters and ethers dissolved in a solvent selected from the class consisting of lower aliphatic alcohols, lower aliphatic ketones, lower aliphatic glycol esters, and lower aliphatic glycol ethers.

6. The method for providing a light-sensitive diazo-type layer on an impervious unsaturated polyester resin surface of a photographic base material which comprises providing on said surface a coat of an amine-formaldehyde resin and a non-drying oil acid-modified phthalic alkyd resin and a solvent-soluble material from the class consisting of cellulose esters, cellulose ethers and shellac, a first overcoat of shellac and a member selected from the class consisting of cellulose esters and cellulose ethers, and a second overcoat of an acrylic ester resin and a member selected from the class consisting of cellulose esters and cellulose ethers, and coating the coated surface with an organic solvent solution of a light-sensitive diazo compound and a member of the class consisting of cellulose esters and ethers, said solvent being a mixture of methanol and butanol and containing a small amount of a lower aliphatic glycol.

7. The method for providing a light-sensitive diazo-type layer on an impervious unsaturated polyester resin surface of a photographic base material which comprises providing on said surface a coat of a urea-melamine-formaldehyde resin and a coconut oil acid-modified trihydric alcohol phthalate alkyd resin and nitrocellulose, a first overcoat of shellac and nitrocellulose, a second overcoat of an acrylic ester resin and nitrocellulose, and an outer coat of a light-sensitive diazo compound and ethyl cellulose.

8. A photographic base material having an impervious unsaturated polyester resin surface, a coat on said surface of an amine-formaldehyde resin and a solvent-soluble material serving to increase the solvent sensitivity of the coat while retaining its adhesiveness, an intermediate coat of shellac and a member selected from the class consisting of cellulose esters and ethers, and an outer coat of a light-sensitive diazo compound and a member selected from the class consisting of cellulose esters and ethers.

9. A photographic base material having an impervious unsaturated polyester resin surface, a coat on said surface of an amine-formaldehyde resin and a member selected from the class consisting of cellulose esters, cel-

lulose ethers, and shellac, an intermediate coat of shellac and a member selected from the class consisting of cellulose esters and ethers, and an outer coat of a light-sensitive diazo compound and a member selected from the class consisting of cellulose esters and ethers.

5 10. A photographic base material having an impervious unsaturated polyester resin surface, a coat on said surface of an amine-formaldehyde resin and a non-drying oil acid-modified phthalic alkyd resin and a member selected from the class consisting of cellulose esters, cellulose ethers, and shellac, an intermediate coat of shellac and a member selected from the class consisting of cellulose esters and ethers, and an outer coat of light-sensitive diazo compound and a member selected from the class consisting of cellulose esters and ethers.

15 11. A dimensionally stable diazotype photographic reproduction material comprising photo-template glass cloth, a coat adhering to a surface thereof of an amine-formaldehyde resin and a non-drying oil acid-modified phthalic alkyd resin and a member selected from the class consisting of cellulose esters, cellulose ethers, and shellac, an intermediate coat of shellac and a member selected from the class consisting of cellulose esters and ethers, and an outer coat of a light-sensitive diazo compound and a member selected from the class consisting of cellulose esters and ethers.

20 12. A dimensionally stable diazotype photographic reproduction material consisting essentially of photo-template glass cloth, a coat adhering to a surface thereof of a urea-melamine-formaldehyde resin and a coconut oil acid-modified trihydric alcohol phthalate alkyd resin and nitrocellulose, a first overcoat of shellac and nitrocellulose adhering to the outer surface of the first-named coat, a second overcoat of an acrylic ester resin and nitrocellulose adhering to the outer surface of the first overcoat, and an outer coat of a light-sensitive diazo compound and ethyl cellulose adhering to the outer surface of the second overcoat.

#### References Cited in the file of this patent

#### UNITED STATES PATENTS

|              |                |       |                |
|--------------|----------------|-------|----------------|
| 40 1,756,400 | Schmidt        | ----- | Apr. 29, 1930  |
| 1,947,160    | Holzwarth      | ----- | Feb. 13, 1934  |
| 1,997,745    | Renker         | ----- | Apr. 16, 1935  |
| 2,140,089    | Marasco        | ----- | Dec. 13, 1938  |
| 2,433,515    | Jahoda         | ----- | Dec. 30, 1947  |
| 2,606,117    | Trojnar        | ----- | Aug. 5, 1952   |
| 2,616,803    | Ravich         | ----- | Nov. 4, 1952   |
| 2,663,640    | Reichel et al. | ----- | Dec. 22, 1953  |
| 2,698,240    | Alles et al.   | ----- | Dec. 28, 1954  |
| 2,718,476    | Eichorn        | ----- | Sept. 20, 1955 |